

# UNITED STATES PATENT OFFICE.

CLEMENT LINWOOD PERKINS, OF PITTSBURGH, PENNSYLVANIA, ASSIGNOR TO METALS RECOVERY COMPANY, OF NEW YORK, N. Y., A CORPORATION OF MAINE

## FLOTATION OF MINERALS.

1,302,966.

Specification of Letters Patent.

Patented May 6, 1919.

No Drawing.

Application filed October 12, 1917. Serial No. 196,121.

*To all whom it may concern:*

Be it known that I, CLEMENT L. PERKINS, a citizen of the United States, residing at Pittsburgh, in the county of Allegheny, 5 State of Pennsylvania, have invented certain new and useful Improvements in the Flotation of Minerals; and I do hereby declare the following to be a full, clear, and exact description of the invention, such as will enable others skilled in the art to which it 10 pertains to make and use the same.

This invention relates to the concentration of minerals, such as sulfid ores and the like (for example, chalco-pyrite with a silicious 15 gangue) by flotation, and is based upon the discovery that improved results can be obtained by carrying out the flotation operation with the addition to the ore or mineral pulp of quinolin, either alone, or with the 20 addition of other agents promoting the flotation. It is not necessary that chemically pure quinolin be used, but the commercial product can be used in its crude unrefined state.

25 In using the quinolin, which is a liquid, it may be added to the ore either alone or in admixture with other agents promoting the flotation, in any suitable manner, so that it will be thoroughly and uniformly distributed throughout the ore pulp. The mixture is then subjected to a flotation operation as in an ordinary Calow cell or in apparatus where the air is incorporated in the ore pulp by mechanical agitation. With some ore 30 pulps it may be desirable to add either small amounts of acids or of alkalis, depending upon the nature of the ore pulp to be treated, but it will be evident that if the ore pulp contains free acid, or if acid is preliminarily added thereto, the free acid should 35 not be present to any such extent as would prejudice or destroy the effect of the quinolin during the flotation operation. The amount of quinolin used may vary somewhat, for example, between one-half pound 40 or less and one and one-half pounds per ton of ore (that is, calculated on the weight of the ore and not on the weight of the ore pulp). It is characteristic of the invention 45 that the froth obtained is readily broken up,

so that any quinolin recoverable from the froth may be used in the treatment of further amounts of ore. That is to say, the circuit water recovered from the concentrate and even that recovered from the tailings 55 contain notable amounts of the quinolin which can be thus returned to the process with resulting economy in the amount required to be used for subsequent operations.

The quinolin may be used alone to promote the flotation operation and high grades 60 of concentrates obtained; and the resulting concentrates can be much more easily separated by filtration than the common concentrates obtained by the use of oil as the flotation agent. The action of the quinolin may, however, be modified by adding other agents 65 (such as oils or non-oleaginous agents) which promote the flotation and which do not prejudicially affect the action of the 70 quinolin.

In applying the quinolin, it may be introduced into the tube mill in which the ore is being ground, or it may be otherwise introduced into the ore pulp in any suitable way, 75 as, for instance, by introducing it into the ore pulp directly into the flotation cell or just before it enters the flotation cell.

What I claim is:

1. The method of effecting the concentration of minerals by flotation, which comprises adding to the mineral pulp a small amount of quinolin, and subjecting the resulting mixture to a flotation operation; substantially as described. 80

2. The method of effecting the concentration of minerals by flotation, which comprises adding to the mineral pulp a small amount of quinolin and other agents promoting the flotation, and subjecting the resulting mixture to a flotation operation; substantially as described. 85

3. The method of effecting the concentration of minerals by flotation, which comprises adding to the mineral pulp a small amount of quinolin and of oil, and subjecting the resulting mixture to a flotation operation; substantially as described. 90

In testimony whereof I affix my signature.

CLEMENT LINWOOD PERKINS.